

Sept. 2, 1924.

1,507,397

R. MOLDENKE

SMELTING OR FUSING METALLIC SUBSTANCES

Filed Dec. 17, 1922

3 Sheets-Sheet 1



INVENTOR  
Richard Moldenke

BY Penrice, Davis, Marvin, & Edmonds

ATTORNEY

Sept. 2, 1924.

1,507,397

R. MOLDENKE

SMELTING OR FUSING METALLIC SUBSTANCES

Filed Dec. 11, 1922

3 Sheets-Sheet 2



INVENTOR  
Richard Moldenke

BY Penick, Davis, Marvin, & Edmunds

ATTORNEY

Sept. 2, 1924.

R. MOLDENKE

1,507,397

SMELTING OR FUSING METALLIC SUBSTANCES

Filed Dec. 11, 1922

3 Sheets-Sheet 3

Fig. 5.



INVENTOR  
Richard Moldenke

BY Penne, Davis, Marvin, & Edmonde

ATTORNEY

Patented Sept. 2, 1924.

## UNITED STATES PATENT OFFICE.

RICHARD MOLDENKE, OF WATCHUNG, NEW JERSEY.

## SMELTING OR FUSING METALLIC SUBSTANCES.

Application filed December 11, 1922. Serial No. 606,045.

*To all whom it may concern:*

Be it known that I, RICHARD MOLDENKE, a citizen of the United States, residing at Watchung, in the county of Somerset, State of New Jersey, have invented certain new and useful Improvements in Smelting or Fusing Metallic Substances; and I do hereby declare the following to be a full, clear, and exact description of the invention, such as will enable others skilled in the art to which it appertains to make and use the same.

This invention relates to the smelting or fusing of metallic substances, and more particularly to the process of smelting or fusing metallic substances in which the metallic substance is subjected in a furnace to the action of heat resulting from the combustion of fluid and solid fuels. The invention has for its object certain improvements in processes of this character.

In the United States patents of Bradley Stoughton, No. 1,117,274, patented November 17, 1914, and No. 1,876,479, patented May 3, 1921, processes of the character to which the present invention relates are described. The essential features of these processes involve the use of as much fluid fuel as practicable to supply the heat required and the minimum quantity of solid fuel. Such processes are of particular importance in localities where solid fuel is scarce or expensive. In the practice of these processes, and the same is true of the present invention, any desirable form of fluid fuel may be used, either gaseous or liquid, as, for example, a combustible gas, either natural or generated, or pulverized fuel, but ordinarily oil is most available and satisfactory. Similarly, any desirable form of solid fuel may be used as, for example, coal or charcoal but ordinarily coke is generally used.

Heretofore in the practice of these processes, it has been customary to blow in the fluid fuel, usually oil, directly with the air blast, either in the same tuyères in the usual position in cupola melting practice, or just a little above this position, but always under or lower than the melting zone of the furnace, that is, the zone of the furnace where the metallic substance fuses or melts. When melting iron, I have found that while this practice produces hot molten metal, nevertheless the motion iron may be oxidized to such an extent as to objectionably and injuriously affect the so-called "life" of the metal. This slight oxidation of the molten

iron raises the "freezing point" of the molten metal as a result of the solution in the iron of an appreciable amount of an oxide of iron. In ordinary foundry practice, such molten iron, when thus slightly oxidized, has to be poured off quickly into molds, otherwise the metal will set in the gates before the molds have been completely filled, thereby materially reducing the number of usable castings produced.

I have discovered that hot molten iron can be produced without objectionable oxidation by heating the metal to near its melting point by heat resulting for the most part from the combustion of the fluid fuel and then raising the temperature of the metal to effect its fusion by heat resulting for the most part from the combustion of the solid fuel appropriately mixed with the metal. Thus, my present invention involves the separate application in different zones or parts of the cupola or other furnace of the heat resulting respectively from the combustion of the fluid fuel and the solid fuel, to the end that the heat resulting from the combustion of the fluid fuel be utilized to preheat the metallic substance, such as iron, while the heat resulting from the combustion of the solid fuel effects the melting or fusion of the metallic substance.

In carrying out my invention, I introduce the heat resulting from the combustion of the fluid fuel into the furnace at a point above the melting zone of the metallic substance. In my preferred practice, the fluid fuel, such as oil, is burned in an independent burner or apparatus and the hot gaseous products resulting therefrom are appropriately conducted to and into the furnace above its melting zone. These hot gaseous products serve to preheat the metallic substance, such as iron, and to bring it to a temperature approaching its melting temperature. In my preferred practice, the zone in which this preheating take place contains insufficient combustion-supporting gas, such as air, oxygen or the like, to support active combustion of the solid fuel mixed with the metallic substance. Having been brought to near its melting temperature, the metallic substance next passes into the melting zone of the furnace where its temperature is raised to effect the desired fusion of the metal by heat resulting from the combustion of the solid fuel admixed with the metallic substance. In the melting zone, active com-

bustion of the solid fuel is insured by introducing into this zone through appropriate tuyères, or the like, a surplus of air, or other appropriate combustion-supporting gas.

The following description, taken in conjunction with the accompanying drawings, will make the invention and the manner of carrying it out in practice clear to those skilled in the art. In the drawings—

Fig. 1 is a sectional elevation of a cupola furnace adapted for the practice of the invention;

Fig. 2 is a diagrammatic view on a reduced scale of the cupola of Fig. 1 operatively connected with an independent burner for the fluid fuel;

Fig. 3 is a sectional plan view of the same on the line 3—3 of Fig. 2;

Figs. 4 and 5 are sectional elevations of modified constructions of cupolas adapted for the practice of the invention; and

Figs. 6 and 7 are detailed views of a peep hole and peep hole cover respectively.

The cupola furnace illustrated in Fig. 1 comprises a steel shell 10 and a fire-brick lining 11 appropriately supported on pillars 12. The usual tap holes or spouts 13 and 14 are provided for tapping off the fused metal and the slag or cinder respectively. A series of tuyères 15 communicate with the interior of the cupola near the lower part thereof. These tuyères are supplied with air or similar combustion-supporting gas through a wind box 16 in communication with an air pipe 17.

A brick flue 18 surrounds the cupola at an appropriate distance above the tuyères 15. A series of ports 19, see Fig. 3, provide communication between the flue 18 and the interior of the cupola. The flue 18 is connected to the combustion chamber of the auxiliary and independent fluid fuel burner 20.

The burner 20 is preferably a fire-brick lined structure provided with a plurality of fluid fuel burners. As illustrated in Fig. 3, these fluid fuel burners consist of pipes 21 for supplying an appropriate fluid fuel such, for example, as crude oil, fuel oil, pulverized fuel, tar, or the like, and pipes 22 for supplying compressed air. A wind box 23 supplied with air from a fan through pipe 24 is associated with each fluid fuel burner 20 and serves to introduce into the combustion chamber of the burner 20 a regulatable blast of air or similar combustion-supporting gas. Man holes 25 and 26 are provided at the top and end respectively of burner 20.

Peep-holes may be provided in the conduit between the combustion chamber of the burner 20 and the flue 18, or in the flue 18 opposite the ports 19, or at any desired point in the combination of apparatus.

The peep-hole, or arrangement for observ-

ing conditions in the interior of the cupola or any part of its appurtenances, consists of a small opening 27 through the shell and firebrick lining within range of a snugly fitting peep-hole cover 28 adapted to be revolved in either a clockwise or counter clockwise direction. The peep-hole cover contains a peep-hole 29 and an opening 30 so positioned that they may be superposed over the opening 27 in the furnace lining by merely turning the peep-hole cover in one direction or the other. The peep-hole 29 contains a transparent heat resisting material, such as mica, and when properly superposed over the opening 27 enables one to view the interior of the apparatus from close range. The opening 30 contains no obstruction and when properly superposed over the opening 27 allows the flame from the apparatus to shoot out thereby enabling the operator to accurately observe the character of the combustion taking place in the apparatus. Any obstruction lodging in opening 27 or ports 19 may be removed by inserting a rod or poker through the opening 30. It will be understood, however, that when no observations are being made the peep-hole cover may be turned so as to close the opening 27 and prevent admission of air to the interior of the apparatus.

The burner 20 may be fired similar to any ordinary fluid burning furnace. The man holes 25 and 26 may be opened to allow sufficient air to enter the burner to support ordinary combustion. Oil from pipe 21 may be atomized by compressed air from pipe 22 and ignited. When the burner walls become red hot and will keep the atomized oil alight, the man holes are closed and proper combustion is brought about and maintained by controlling the amount of air supplied from a fan, not shown, to the wind box 23. The hot products of combustion from the burner 20 pass into the flue 18 and thence to the cupola through the ports 19. An air blast is then forced into the cupola through the tuyères 15 near the bottom thereof and supports the combustion of the solid fuel, which, in turn, supplies sufficient additional heat to melt and superheat the metal for pouring into moulds.

The cupola is charged periodically with mixtures of pig or scrap metal, fuel and, if necessary, also, with slag-forming materials. I prefer to charge the cupola with alternate layers of solid fuel and pig or scrap metal. As the apparatus continues in operation charges of solid fuel and metal pass progressively downward in the cupola, first through the oil-heat position, or preheating zone, where the solid fuel and metal is raised by the hot products of combustion of the fluid fuel to a temperature just under the melting temperature of the metal, and then into the melting zone where the metal

is fused and the drops fall and are superheated for pouring into molds by the combustion of the solid fuel. The thus superheated molten metal may be tapped from the 5 crucible of the cupola from time to time and withdrawn through the tap or spout 13 while the slag may be drawn off through the tap or spout 14.

In accordance with the present invention 10 any surplus of air above the melting zone is particularly to be avoided. Any surplus air in this zone of the cupola is likely to ignite the solid fuel between the metal charges and furnish sufficient heat to melt the metal. 15 Consequently, I maintain the oil flame a little smoky by using just sufficient compressed air (about 80 to 100 pounds per square inch) to properly atomize the oil to form an oil fog, and take such additional 20 air as may be necessary for the desired combustion from a fan.

I prefer to take this additional air supply from a fan in preference to the positive blower generally used for supplying the air 25 used to burn the coke charges in a cupola. The air supply from a fan can be easily shut off or on by a blast gate so that the quantity of air used may be regulated between a maximum and minimum with ease while the 30 fan remains revolving at full speed all the time. The positive blower which cannot be regulated so easily is preferably used for the air supply to bring about combustion of the solid fuel and should remain at constant volume throughout the melt and 35 should be shut off entirely, if shut off at all, and then only, when the iron comes too fast to be used readily. Under such conditions it is possible to give more or less oil with 40 more or less air from a fan as may be desired or necessary and yet introduce no more heat above the melting zone than may be necessary to bring the metal to a temperature just short of actual melting.

45 The character of the combustion of the fluid fuel may be observed by properly superposing the opening 30 over the opening 27 and allowing the flame to shoot out. I have discovered that the best and most 50 economical results may be obtained when the combustion of the fluid fuel is regulated so as to secure a red or yellow flame with just a slight smoky tip.

55 In Fig. 4 I have illustrated a modified form of apparatus adapted for the practice of the invention. In this apparatus the independent burner for supplying the cupola with hot products of combustion from fluid fuel is entirely eliminated. In a position 60 corresponding to the position occupied by the flue 18 of the preferred form of apparatus (illustrated in Fig. 1) I have provided an annular combustion chamber 31 for fluid fuel as an integral part of the cupola to 65 which the fluid fuel is supplied from the oil

supply pipe 21, the compressed air pipe 22, and the wind box 23.

The character of the oil flame is controlled and maintained in the same manner as the oil flame in the burner 20 of the preferred 70 form of apparatus. The hot products of combustion of the fluid fuel pass from the combustion chamber 31 through the ports 19 into the preheating zone of the cupola. In all respects the operation of this apparatus is similar to the preferred form of apparatus and will be understood, it is believed, from the foregoing description.

A further modified form of apparatus is 75 illustrated in Fig. 5. In this apparatus the wind box 23 is positioned in operative association with the ports 19, the fluid fuel and compressed air being supplied directly to the cupola by the oil pipe 21 and compressed air pipe 22. The fuel mixture passes 80 through the ports 19 into the preheating zone of the cupola where it is ignited and burned as in the forms of apparatus previously described.

Heretofore in the practice of smelting or 85 fusing operations of the type described some difficulty has been experienced affecting the so-called life of the metal. By the practice of the present invention I obtain a superheated molten metal admirably 90 suited for molding purposes. The cupola melting process provides two definite zones of heat application. The metal is heated first by the heat generated from the combustion of the fluid fuel to a degree approaching 95 the melting temperature of the metal and under conditions such as not to cause subsequent trouble from lack of life when the red or white metal is properly melted in the regular melting zone by the 100 heat generated from the combustion of the solid fuel.

Inasmuch as most of the heat used in the 105 cupola is utilized to raise the temperature of the metal charges to near their melting point, and a much smaller portion of the 110 heat is required to actually melt and superheat the metal, the importance of thus preheating the metal by the combustion of 115 fluid fuel is apparent.

Throughout this specification and the 120 appended claims, I have, for the sake of simplicity, spoken of air in a broad sense to include any equivalent or appropriate combustion-supporting gas or gases. By surplus 125 of air is to be understood such an amount of air or equivalent combustion-supporting gas as will support active combustion of the solid fuel in the melting zone of the furnace. As will be understood from the 130 foregoing description, this surplus of air should be so regulated and correlated to the amount of solid fuel in the melting zone 135 that no substantial excess of combustion-supporting gas enters the preheating zone 140

with the gaseous products from the melting zone. The combustion of the fluid fuel without surplus air involves so regulating the combustion of the fluid fuel that the resulting hot gaseous products of combustion contain little, and preferably no, surplus of combustion-supporting gas. Where the optimum advantages of the invention are realized, as in my preferred practice, 10 these conditions and factors are so regulated and correlated that the preheating zone of the furnace contains insufficient combustion-supporting gas to support active combustion of the solid fuel as it passes through 15 this zone.

When water vapor comes into contact with solid iron there is formed a coat of iron oxide corresponding somewhat to rust. As this coated, or rusted, solid iron descends 20 into the melting zone of the furnace, there is either the chance of a reduction of the iron oxide by the carbon monoxide (CO) gas on the way down, or else in the melting 25 of the iron the oxide is in a measure cared for by the slag, or else the amount is so little that it does not affect the product any more than rust does in ordinary melting. In other words, probably none of the oxide gets into the molten metal, or only a negligible 30 amount, so that the freezing point will not be materially affected.

On the other hand, when water vapor comes into contact with the drops of molten metal in the forming, the melting metal being in contact with the water vapor an appreciable time before the drop falls off the still solid piece of iron, there is a chance for the continual solution of the iron oxide formed on the surface of the forming drop 35 of molten metal and thus a comparatively large amount of dissolved iron oxide in the metal raises the freezing point. The result is that very hot molten metal, by setting too fast, will not give proper castings when 40 poured into molds. In the melting zone proper there is no opportunity for a reduction of iron oxide by carbon monoxide gas, as may take place higher up in the furnace. 45 There is no carbon monoxide gas in the melting zone, or in any event there should be little, if any, such gas that low down in the furnace. The carbon monoxide gas is formed higher up and at these higher levels 50 may possibly reduce rust to metallic iron. 55 It is for these reasons that, in accordance with my present invention, the liquid fuel is introduced above the melting zone of the furnace. What I aim to achieve is to prevent the formation of iron oxide by water vapor where this oxide cannot be reduced, 60 but on the other hand remains and dissolves in the molten metal with the hereinbefore mentioned disadvantages.

I claim:

1. The improvement in the process of

smelting or fusing metallic substances in which the metallic substance is subjected in a furnace to the action of heat resulting from the combustion of fluid and solid fuels, which comprises so adjusting or arranging 70 the supply of fluid and solid fuels and the air or other combustion-supporting gas or gases that the products of combustion of the fluid fuel shall not come in contact with the molten metal.

2. The improvement in the process of smelting or fusing metallic substances in which the metallic substance is subjected in a furnace to the action of heat resulting from the combustion of fluid and solid fuels, which 75 comprises supplying the heat of combustion of fluid fuel to an appropriate mixture of metallic substance and solid fuel and thereafter bringing the metallic substance to an appropriate molten condition by heat derived solely from the combustion of the solid fuel.

3. The improvement in the process of smelting or fusing metallic substances in which the metallic substance is subjected in 80 a furnace to the action of heat resulting from the combustion of fluid and solid fuels, which comprises supplying the heat of combustion of fluid fuel without surplus air to an appropriate mixture of metallic substance 85 and solid fuel, and thereafter bringing the metallic substance to an appropriate molten condition by heat derived solely from the combustion of the solid fuel in the presence of an appropriate amount of air.

4. The improvement in the process of smelting or fusing metallic substances in which the metallic substance is subjected in a furnace to the action of heat resulting from the combustion of fluid and solid fuels, which 90 comprises supplying the heat of combustion of fluid fuel to an appropriate mixture of metallic substance and fuel in a pre-heating zone, and thereafter bringing the metallic substance to an appropriate molten condition in a melting zone by heat derived solely from the combustion of the solid fuel.

5. The improvement in the process of smelting or fusing metallic substances in which the metallic substance is subjected in a 95 furnace to the action of heat resulting from the combustion of fluid and solid fuels, which comprises supplying the heat of combustion of fluid fuel without surplus air to an appropriate mixture of metallic substance and fuel in a preheating zone, and thereafter bringing the metallic substance to an appropriate molten condition in a melting zone by heat derived solely from the combustion of the solid fuel in the presence of an appropriate amount of air.

6. The improvement in the process of smelting or fusing metallic substances in which the metallic substance is subjected in a furnace to the action of heat resulting 100

from the combustion of fluid and solid fuels which comprises progressively passing the metallic substance appropriately mixed with solid fuel through a preheating zone maintained for the most part by the combustion of fluid fuel at a temperature slightly below the melting temperature of the metallic substance and then passing the metallic substance thus preheated to a temperature approaching its melting temperature through a melting zone maintained for the most part by the combustion of said solid fuel at a temperature above its melting temperature.

7. The improvement in the process of smelting or fusing metallic substances in which the metallic substance is subjected in a furnace to the action of heat resulting from the combustion of fluid and solid fuels which comprises progressively passing the metallic substance appropriately mixed with solid fuel through a preheating zone maintained for the most part by the combustion of fluid fuel without surplus air at a temperature slightly below the melting temperature of the metallic substance and then passing the metallic substance thus preheated to a temperature approaching its melting temperature through a melting zone maintained for the most part by the combustion of said solid fuel in the presence of an appropriate amount of air at a temperature above the melting temperature of the metallic substance.

8. The improvement in the process of smelting or fusing metallic substances in which the metallic substance is subjected in a furnace to the action of heat resulting from the combustion of fluid and solid fuels which comprises progressively passing the metallic substance appropriately mixed with solid fuel through a preheating zone and a melting zone, said preheating zone deriving its heat for the most part from the combustion of liquid fuel and said melting zone deriving its heat for the most part from the combustion of said solid fuel.

9. The improvement in the process of smelting or fusing metallic substances in which the metallic substance is subjected in a furnace to the action of heat resulting from the combustion of fluid and solid fuels which comprises progressively passing the metallic substance appropriately mixed with solid fuel through a preheating zone and a melting zone, said preheating zone deriving its heat for the most part from the combustion of liquid fuel without surplus air and said melting zone deriving its heat for the most part from the combustion of said solid fuel in the presence of an appropriate amount of air.

10. The improvement in the process of smelting or fusing metallic substances in which the metallic substance is subjected in a furnace to the action of heat resulting

from the combustion of fluid and solid fuels which comprises progressively passing the metallic substance appropriately mixed with solid fuel through a preheating zone whose temperature approaches but does not reach the melting temperature of the metallic substance and through a melting zone whose temperature exceeds the melting temperature of the metallic substance, said preheating zone deriving its heat for the most part from the combustion of liquid fuel and said melting zone deriving its heat for the most part from the combustion of said solid fuel.

11. The improvement in the process of smelting or fusing metallic substances in which the metallic substance is subjected in a furnace to the action of heat resulting from the combustion of fluid and solid fuels which comprises progressively passing the metallic substance appropriately mixed with solid fuel through a preheating zone whose temperature approaches but does not reach the melting temperature of the metallic substance and through a melting zone whose temperature exceeds the melting temperature of the metallic substance, said preheating zone deriving its heat for the most part from the combustion of liquid fuel without surplus air and said melting zone deriving its heat for the most part from the combustion of said solid fuel in the presence of an appropriate amount of air.

12. The improvement in the process of smelting or fusing metallic substances in which the metallic substance is subjected in a furnace to the action of heat resulting from the combustion of fluid and solid fuels which comprises bringing the metallic substance to substantially its melting temperature by heat resulting for the most part from the combustion of fluid fuel and then effecting the fusion of the metallic substance by heat resulting for the most part from the combustion of solid fuel appropriately admixed therewith.

13. The improvement in the process of smelting or fusing metallic substances in which the metallic substance is subjected in a furnace to the action of heat resulting from the combustion of fluid and solid fuels which comprises bringing the metallic substance to substantially its melting temperature by heat resulting for the most part from the combustion of fluid fuel without surplus air and then effecting the fusion of the metallic substance by heat resulting for the most part from the combustion in the presence of an appropriate amount of air of solid fuel appropriately mixed with the metallic substance.

14. The improvement in the process of smelting or fusing metallic substances in which the metallic substance is subjected in a furnace to the action of heat resulting

from the combustion of fluid and solid fuels which comprises progressively passing the metallic substance appropriately mixed with solid fuel downwardly through a preheating zone and a melting zone of the furnace, said preheating zone being heated for the most part by the hot gaseous products resulting from the combustion exteriorly of the furnace and its direct appurtenances of fluid fuel and said melting zone being heated for the most part by heat resulting from the combustion of said solid fuel.

15. The improvement in the process of smelting or fusing metallic substances in which the metallic substance is subjected in a furnace to the action of heat resulting from the combustion of fluid and solid fuels which comprises progressively passing the metallic substance appropriately mixed with solid fuel downwardly through a preheating zone and a melting zone of the furnace, said preheating zone being heated for the most part by the hot gaseous products resulting from the combustion exteriorly of the furnace and its direct appurtenances of fluid fuel without excess of air, and said melting zone being heated for the most part by heat resulting from the combustion of said solid fuel in the presence of an appropriate amount of air.

16. The improvement in the process of smelting or fusing metallic substances in which the metallic substance is subjected in a furnace to the action of heat resulting from the combustion of fluid and solid fuels which comprises progressively passing alternate layers of the metallic substance and solid fuel downwardly through a preheating zone and a melting zone, subjecting the metallic substance as it passes through the preheating zone to heat resulting for the most part from the combustion of fluid fuel, said preheating zone containing insufficient combustion supporting gas to support active combustion of said solid fuel as it passes therethrough, and fusing the preheated metallic substance in said melting zone by heat resulting for the most part from the active combustion of said solid fuel in the presence of an appropriate amount of air.

17. The improvement in the process of smelting or fusing metallic substances in which the metallic substance is subjected in a furnace to the action of heat resulting

from the combustion of fluid and solid fuels which comprises progressively passing alternate layers of the metallic substance and solid fuel downwardly through a preheating zone and a melting zone, subjecting the metallic substance as it passes through the preheating zone to the hot gaseous products resulting from the combustion exteriorly of the furnace and its direct appurtenances of fluid fuel, said preheating zone containing insufficient combustion supporting gas to support active combustion of said solid fuel as it passes therethrough, and fusing the preheated metallic substance in said melting zone by heat resulting for the most part from the active combustion of said solid fuel in the presence of an appropriate amount of air.

18. The improvement in the process of smelting or fusing metallic substances in which the metallic substance is subjected in a furnace to the action of heat resulting from the combustion of fluid and solid fuels which comprises bringing the metallic substance to substantially its melting temperature by the hot gaseous products resulting from the combustion exteriorly of the furnace and its direct appurtenances of fluid fuel, and then effecting the fusion of the metallic substance by heat resulting for the most part from the combustion of solid fuel appropriately mixed therewith.

19. The improvement in the process of smelting or fusing metallic substances in which the metallic substance is subjected in a furnace to the action of heat resulting from the combustion of fluid and solid fuels which comprises bringing the metallic substance appropriately mixed with solid fuel to substantially its melting temperature by the hot gaseous products resulting from the combustion exteriorly of the furnace and its direct appurtenances of fluid fuel, maintaining insufficient combustion-supporting gas in contact with the solid fuel admixed with the metallic substance while the latter is undergoing the aforementioned preheating to support active combustion of said solid fuel, and subsequently effecting the fusion of the metallic substance by heat resulting for the most part from the active combustion in the presence of an appropriate amount of air of said solid fuel.

In testimony whereof I affix my signature.  
RICHARD MOLDENKE.